

Dec. 27, 1927.

1,654,046

L. KAHL

PROCESS FOR THE PRODUCTION OF ARC LIGHT ELECTRODES

Filed May 31, 1923



*Inventor*

*L. Kahl*  
*by*

*W. S. Evans*  
*Attorney.*

Patented Dec. 27, 1927.

## UNITED STATES PATENT OFFICE.

LEOPOLD KAHL, OF BERLIN-DAHLEM, GERMANY, ASSIGNOR TO RÜTGERSWERKE AK-  
TIENGESELLSCHAFT, ABTEILUNG PLANIWERKE, OF BERLIN, GERMANY.

## PROCESS FOR THE PRODUCTION OF ARC-LIGHT ELECTRODES.

Application filed May 31, 1923, Serial No. 642,670, and in Germany June 9, 1922.

Arc-light electrodes have hitherto been manufactured by intimately mixing carbonaceous material, such as coke, soot, retort graphite, or the like, with a binding agent such, for example, as tar oil, tar, syrup, starch, and the like, in mixing machines. After being mixed the material is kneaded in edge-mills or calenders in order to obtain as uniform and plastic a consistency as possible. The mass obtained is then by preliminary compression formed into balls or masses, which are of such cross-section that they will subsequently fit into the cylinder of a hydraulic press. The preliminary compression is effected either in ordinary presses or in hydraulic presses. The ball or mass is then put into the cylinder of a hydraulic press and extruded through a mouth-piece, the opening of which is of the same shape as the finished carbon. The raw carbon is then finished and afterwards burnt in order to carbonize the binding agent, and is then ready for sale.

This method, which has been the one hitherto employed, was, however, attended by a number of disadvantages. Even with the most intimate working up of the raw materials it was impossible by this method to remove air imprisoned in the mass. The material was plastic and possessed all the properties of a true fluid—that is to say, its volume increased upon relaxation of the pressure in accordance with its increasing elasticity. This was particularly manifest in the moulding of the carbon in the hydraulic press. Further, the density of the compressed mass could not be increased by a given pressure, as the elasticity of the mass acted in opposition to the pressure and the article extruded from the mouth-piece was of greater cross-section than the mouth-piece itself. The carbon makers, however, sought to make the carbon more dense and less porous, as upon the density of the carbon not only depends the combustion thereof, but also (in the case of the so-called homogeneous effect-carbons that contain the illuminating salts intimately disseminated throughout the whole transverse section) the radiation of the light. It has therefore also been suggested not to extrude carbons or electrodes in the form of a cord or string from an extruding press but to press them separately in moulds; and it has also been suggested to press the raw carbon extruded from an hydraulic press in the form of a cord in a mould.

Both these methods are, however, not only very uneconomical, as pressing in moulds is expensive and takes up much time, but they also suffer from the disadvantage that the openings which are provided in the moulds for the escape of air and gases become very easily choked up, whereby the object aimed at, namely that of making the electrodes or carbons denser, cannot be attained.

These disadvantages are overcome according to the present invention by the fact that in the preparation of the raw material it is made at the very commencement as dense as it is possible to make it and this density is increased at each further operation. This is attained in the first instance by a complete removal of the air from the crude mass, which is effected by compression of the masses or balls thereof, while the masses or balls are subjected to a vacuum. By such means the mass or masses are deprived of air and are also compressed or consolidated. This mass from which the air has been thus removed is then ejected from the press and rolled out as thinly as possible on calenders. The rolled-out thin layers are then superposed and again subjected to mechanical pressure under a vacuum the mass being simultaneously given the form of the lumps which fit the moulding cylinder. The crude mass or the masses produced in the respective stages of the process may be subject to compression in any type of press, it being only necessary that the mould space in which the mass to be compressed is passed should be put into communication as by means of a pipe with a vacuum pump or a vessel in which a vacuum is maintained. The accompanying drawing illustrates diagrammatically such a press in which the mass to be deprived of air and to be compressed is placed within a cylinder *b* in which operates the plunger of an hydraulic press with power cylinder *a*. In the operation of the press the mass is subjected to pressure by the plunger on movement of the piston within the power cylinder *a* and simultaneously the mass is subjected to a vacuum exerted through the pipe *f* by the vacuum pump *d*. A pressure pump *c* is also connected to the cylinder *b* by the pipe *e* and is advantageously employed to apply fluid pressure to the moulded mass upon the completion of the

- movement and the retraction of the plunger to facilitate the removal of the moulded mass. The pipes *e* and *f* are provided with closure members *g* and *h* respectively for the control of the action of the pipes *d* and *c* as desired. The simultaneous use of a vacuum and mechanical pressure also enables the amount of binding agent requisite to be reduced, thereby likewise increasing the strength of the product. In this way the masses or balls are deprived of a portion of their elasticity, and it is now possible to use in the hydraulic extrusion press pressures which have hitherto been impossible in the production of artificial carbons. The subsequent process of treatment employed is carried out in the usual way, but it is advisable, in order to render the carbon still denser, to impregnate it before burning with tar oil in the usual way under vacuum and pressure, whereby the last remaining pores become filled up with tar coke when the carbons are subsequently burned. Suitable means for the purpose are described by Dr. Julius Zellner in his book "Die künstlichen Kohlen für elektrotechnische und elektro-chemische Zwecke, ihre Herstellung und Prüfung" (published by Julius Springer, Berlin 1903).
- Instead of the tar now commonly employed colloidal carbon may be employed both in the preparation of the mixture and also in the impregnation of the crude carbon which enables a minimum amount of binding agent to be used.
- I claim:
1. A process for the manufacture of carbon electrodes for arc-lighting consisting in subjecting a plastic mass of raw material and binding agent to compression in a vacuum, then moulding bodies in the form of elec-  
trodes from the mass thus treated, and then subjecting the said bodies to burning, substantially as described.
  2. A process for the manufacture of carbon electrodes for arc-lighting consisting in subjecting a plastic mass of raw material and binding agent repeatedly to compression in a vacuum, the compressed mass being broken down between successive stages of compression and moulding bodies from the mass produced, in the form of electrodes, substantially as described. 45
  3. A process for the manufacture of carbon electrodes for arc-lighting consisting in subjecting a plastic mass of raw material and binding agent to compression in a vacuum, then rolling out the mass produced into thin layers and then again compressing the mass rolled out, substantially as described. 55
  4. A process for the manufacture of carbon electrodes for arc-lighting consisting in subjecting a plastic mass of raw material and binding agent to compression in a vacuum, impregnating the mass with a filling substance such as tar oil under vacuum and pressure, then moulding the plastic mass into the form of bodies adapted for use as electrodes, and then subjecting the said bodies to burning, substantially as described. 60
  5. A process for the manufacture of carbon electrodes for arc-lighting consisting in subjecting a plastic mass of raw material and binding agent to compression in a vacuum, then rolling out the mass produced into thin layers and then subjecting the mass so treated to further compression in a vacuum and then moulding from the mass produced bodies in the form of electrodes, substantially as described. 65

LEOPOLD KAHL.